# EUROPEAN PATENT SPECIFICATION

(11) **EP 1 431 051 B1**
(45) Date of publication and mention of the grant of the patent: **11.02.2009**
(21) Application number: 03078824.4
(22) Date of filing: 04.12.2003
(51) Int. Cl.: B41M 5/00

(54) **Ink jet recording element and printing method**
Tintenstrahlaufzeichnungselement und Druckverfahren
Elément d'enregistrement par jet d'encre et méthode d'impression

(30) Priority: 16.12.2002 US 320293; 16.12.2002 US 320206
(43) Date of publication of application: 23.06.2004
(73) Proprietor: Eastman Kodak Company, Rochester NY 14650-2201 (US)
(72) Inventor: Chu, Lixin, c/o Eastman Kodak Company, Rochester, New York 14650-2201 (US); Shaw-Klein, Lori J., c/o Eastman Kodak Company, Rochester, New York 14650-2201 (US); Ruschak, Kenneth J., c/o Eastman Kodak Company, Rochester, New York 14650-2201 (US); Gallo, Elizabeth A., c/o Eastman Kodak Company, Rochester, New York 14650-2201 (US); Vargas, Christine M., c/o Eastman Kodak Company, Rochester, New York 14650-2201 (US); Salerno, Charles, c/o Eastman Kodak Company, Rochester, New York 14650-2201 (US)
(74) Representative: Haile, Helen Cynthia

(56) References cited:
- EP-A- 0 983 867
- EP-A- 1 184 192
- EP-A- 1 184 194
- WO-A-01/70509
- US-B1- 6 485 812

## Description

This invention relates to an ink jet recording element and printing method, more particularly to an ink jet recording element containing a polymeric network.

In a typical ink jet recording or printing system, ink droplets are ejected from a nozzle at high speed towards a recording element or medium to produce an image on the medium. The ink droplets, or recording liquid, generally comprise a recording agent, such as a dye or pigment, and a large amount of solvent. The solvent, or carrier liquid, typically is made up of water and an organic material such as a monohydric alcohol, a polyhydric alcohol or mixtures thereof.

An ink jet recording element typically comprises a support having on at least one surface thereof an ink-receiving or image-receiving layer, and includes those intended for reflection viewing, which have an opaque support, and those intended for viewing by transmitted light, which have a transparent support.

An important characteristic of ink jet recording elements is their need to dry quickly after printing. To this end, porous recording elements have been developed which provide nearly instantaneous drying as long as they have sufficient thickness and pore volume to effectively contain the liquid ink.

Porous inorganic particles, such as silica gel, precipitated silica and clays are widely used in ink jet recording elements because of their highly absorptive properties. For example, EP 0 739 747 A2 and U.S. Patents 5,965,244; 6,114,022 and 6,140,406 disclose porous image-receiving layers containing silica gel and/or precipitated silica. However, these types of image-receiving layers often have low mechanical strength or coating integrity due to weak interactions between the porous particles and, therefore, the image-receiving layer can be easily removed from the support upon which it was coated.

U.S. Patent 5,510,004 relates to the use of polymers and copolymers of N, N-diallyl-3-hydroxyazetidinium salts as agents for improving the wet strength of paper. However, there is no disclosure of using these polymers in an image-receiving layer for an ink jet recording element.

U.S. Patent 6,409,334 discloses the use of an amino-silane compound and inorganic silica colloidal particles combined with a wet-strength polymer having a reactive azetidinium group in producing an image-receiving layer for an ink jet recording element. However, there is no disclosure of using a non-latex polymeric binder that would react with the azetidinium group such that the integrity of the image-receiving layer would be greatly enhanced. Poly(vinyl alcohol) binder is used in other examples that do not include the wet-strength polymer or amino-silane compound.

US-B-6485812 discloses an inkjet recording sheet that comprises inorganic particles, binder resin, and tetraalkoxytitanium, the latter reacting with functional groups having active hydrogen, leading to improved water resistance and scratch resistance as well as less beading.

It is an object of this invention to provide an ink jet recording element that has good image quality with excellent dry time. It is another object of the invention to provide an ink jet recording element having an image-receiving layer of good integrity and sufficient waterfastness.

Still another object of the invention is to provide a printing method using the above-described element.

These and other objects are achieved in accordance with the invention which comprises an ink jet recording element comprising a support having thereon an image-receiving layer comprising a polymeric network formed by a chemical reaction between a wet strength polymer, amino-functionalized inorganic particles and a hydrophilic polymer other than a wet strength polymer, wherein said wet-strength polymer contains at least one highly reactive group comprising an azetidinium or an epoxide, said amino-functionalized inorganic particles comprise silica gel, precipitated silica, or silicates and being obtainable by chemical bond formation between inorganic particles and an amino-functionalized silane coupling agent, and the hydrophilic polymer is poly(vinyl alcohol) present in the image-receiving layer in an amount of from 30 to 70% by weight, wherein the dry thickness of the image-receiving layer ranges from 5 to 30 µm.

By use of the invention, an ink jet recording element is obtained that has a good image quality with an excellent dry time. In addition, the ink jet recording element can be made with a desired coating integrity and waterfastness.

Another embodiment of the invention relates to an ink jet printing method comprising the steps of:
A) providing an ink jet printer that is responsive to digital data signals;
B) loading the printer with the ink jet recording element described above;
C) loading the printer with an ink jet ink composition; and
D) printing on the ink jet recording element using the ink jet ink in response to the digital data signals.

As noted above, the image-receiving layer contains a wet-strength polymer or resin. These materials are well known in the paper and pulp industry. These polymers impart wet strength to paper by crosslinking with cellulose, and subsequently self-crosslinking with the fiber structure of the paper web. Useful wet-strength polymers are cationic and water soluble, yet form a water insoluble network with cellulose. Wet-strength polymers are capable of crosslinking with a variety of organic materials other than cellulose and derivatives, including carboxylated and hydroxylated latexes, poly(vinyl alcohol), amine-containing compounds, alginate, polyacrylates, gelatin, starch, and their derivatives.

The wet-strength polymers are polymers prepared by reacting a polyamine or an amine-containing backbone polymer with an epoxide possessing a second functional group, such as an epichlorohydrin, in water. The result is a polymer containing either one or two highly reactive groups: the azetidinium and the epoxide. Such polymers are well known in the art of polymer chemistry, and are available, for example, as the Kymene® series from Hercules Inc. Especially preferred is Kymene® 557LX. The image-receiving layer of the present invention contains the wet strength polymer in a preferred amount of from 1 to 10% by weight.

The amino-functionalized inorganic particles are prepared by chemical bond formation between inorganic particles and amino-functionalized silane coupling agents. This chemistry is well known in the art of organosilane chemistry, and is described in, for example, "Silicon Compounds: Register and Review", 5th Edition, available from United Chemical Technologies, Inc. This reference describes the theory and methods for effecting chemical bond formation, and how to select the appropriate inorganic particles and coupling agents for a particular use.

In a preferred embodiment of the invention, the amino-functionalized inorganic particles are prepared by combining an amino-functionalized silane coupling agent and inorganic particles in a ratio of from 1:5 to 1:100.

The inorganic particles are porous silica particles such as silica gel, precipitated silica, and silicates.

In another preferred embodiment, the amino-functionalized silane coupling agent has the formula:

(R₁)ₓSi(OR₂)_{y}(R₃)_{z}

wherein:
each R₁ independently represents an alkyl or aryl group, and at least one R₁ is substituted with at least one amino group, such as NH₂(CH₂)₃, NH₂(CH₂)₄, NH₂(CH₂)₅, NH₂(CH₂)₆, NH₂(CH₂)₂NH(CH₂)₂, NH₂(CH₂)₃NH(CH₂)₂, NH₂(CH₂)₂NH(CH₂)₃, NH₂(CH₂)₃NH(CH₂)₃, NH₂(CH₂)₂NH(CH₂)(C₆H₄)(CH₂)₂, NH₂(CH₂)₆NH(CH₂)₃, or NH₂(CH₂)₃OC(CH₃)₂CH=CH;
each R₂ independently represents an alkyl or aryl group, such as methyl, ethyl, 2-ethylhexyl, methoxyethoxyethyl, or trimethylsilyl;
each R₃ is an alkyl group such as methyl, ethyl, propyl or isopropyl;
x is from 1 to 3;
y is from 1 to 3;
z may be 0, 1 or 2; and
the sum of x, y and z is equal to 4.

In another preferred embodiment of the invention, the coupling agent is 3-aminopropyltrimethoxysilane or N-(2-aminoethyl)-3-aminopropylmethyldimethoxysilane. In another preferred embodiment of the invention, between 1 and 20% by weight of the inorganic particles used in the image-receiving layer are reacted with the amino-functionalized silane coupling agent.

The hydrophilic polymer other than a wet-strength polymer which may be used in the invention is poly(vinyl alcohol). The hydrophilic polymer other than a wet-strength polymer is present in the image-receiving layer in an amount of from 30 to 70% by weight.

The ink jet recording element of the invention may also contain other particles such as those described above which are used in preparing the amino-functionalized inorganic particles. These other particles may be used in an amount of from 10 to 70% by weight of the image-receiving layer. In a preferred embodiment of the invention, the ratio of amino-functionalized particles to the other particles is from 1:5 to 1:100.

Also present in the image-receiving layer is one or more mordanting species or polymers. The mordant may be water soluble or water insoluble such as a soluble polymer, a charged molecule, or a crosslinked dispersed microparticle. The mordant can be non-ionic, cationic or anionic. In one embodiment, the mordant is a water soluble cationic mordant. In a preferred embodiment, the mordant is poly(diallyldimethylammonium chloride). The amount of mordant present is typically up to 10% by weight.

The dry thickness of the image-receiving layer ranges from 5 to 30 µm, preferably from 7 to 20 µm. The coating thickness required is determined through the need for the coating to act as a sump for absorption of ink solvent and the need to hold the dye or pigment colorant near the coating surface.

The support for the ink jet recording element used in the invention can be any of those usually used for ink jet receivers, such as resin-coated paper, paper, polyesters, or microporous materials such as polyethylene polymer-containing material sold by PPG Industries, Inc., Pittsburgh, Pennsylvania under the trade name of Teslin ®, Tyvek ® synthetic paper (DuPont Corp.), and OPPalyte® films (Mobil Chemical Co.) and other composite films listed in U.S. Patent 5,244,861. Opaque supports include plain paper, coated paper, synthetic paper, photographic paper support, melt-extrusion-coated paper, and laminated paper, such as biaxially oriented support laminates. Biaxially oriented support laminates are described in U.S. Patents 5,853,965; 5,866,282; 5,874,205; 5,888,643; 5,888,681; 5,888,683; and 5,888,714. These biaxially oriented supports include a paper base and a biaxially oriented polyolefin sheet, typically polypropylene, laminated to one or both sides of the paper base. Transparent supports include glass, cellulose derivatives, e.g., a cellulose ester, cellulose triacetate, cellulose diacetate, cellulose acetate propionate, cellulose acetate butyrate; polyesters, such as poly(ethylene terephthalate), poly(ethylene naphthalate), poly(1,4-cyclohexanedimethylene terephthalate), poly(butylene terephthalate), and copolymers thereof; polyimides; polyamides; polycarbonates; polystyrene; polyolefins, such as polyethylene or polypropylene; polysulfones; polyacrylates; polyetherimides; and mixtures thereof. The papers listed above include a broad range of papers, from high end papers, such as photographic paper to low end papers, such as newsprint.

The support used in the invention may have a thickness of from 50 to 500 µm, preferably from 75 to 300 µm. Antioxidants, antistatic agents, plasticizers and other known additives may be incorporated into the support, if desired.

Coating compositions employed in the invention may be applied by any number of well known techniques, including dip-coating, wound-wire rod coating, doctor blade coating, gravure and reverse-roll coating, slide coating, bead coating, extrusion coating, curtain coating and the like. Known coating and drying methods are described in further detail in Research Disclosure no. 308119, published Dec. 1989, pages 1007 to 1008. After coating, the layers are generally dried by simple evaporation, which may be accelerated by known techniques such as convection heating.

To improve colorant fade, UV absorbers, radical quenchers or antioxidants may also be added to the image-receiving layer as is well known in the art. Other additives include adhesion promoters, rheology modifiers, biocides, lubricants, dyes, optical brighteners, matte agents, antistatic agents, etc.

The coating composition can be coated so that the total solids content will yield a useful coating thickness, and for particulate coating formulations, solids contents from 10-60% by weight are typical.

Ink jet inks used to image the recording elements of the present invention are well known in the art. The ink compositions used in ink jet printing typically are liquid compositions comprising a solvent or carrier liquid, dyes or pigments, humectants, organic solvents, detergents, thickeners, preservatives, and the like. The solvent or carrier liquid can be solely water or can be water mixed with other water-miscible solvents such as polyhydric alcohols. Inks in which organic materials such as polyhydric alcohols are the predominant carrier or solvent liquid may also be used. Particularly useful are mixed solvents of water and polyhydric alcohols. The dyes used in such compositions are typically watersoluble direct or acid type dyes. Such liquid compositions have been described extensively in the prior art including, for example, U.S. Patents 4,381,946; 4,239,543 and 4,781,758.

Although the recording elements disclosed herein have been referred to primarily as being useful for ink jet printers, they also can be used as recording media for pen plotter assemblies. Pen plotters operate by writing directly on the surface of a recording medium using a pen consisting of a bundle of capillary tubes in contact with an ink reservoir.

The following example further illustrates the invention.

### Element 1 of the Invention

A coating composition was prepared by mixing together 100 g of 6 µm silica gel Gasil® 23F (INEOS Silicas) and 420 g of water in a glass container. Then, 10 g of 3-aminopropyltrimethoxysilane (United Chemical Technologies, Inc.) was added under vigorous stirring. After stirring for one hour, 170 g of poly(vinyl alcohol) Gohsenol® GH-03 (Nippon Gohsei Co. Ltd.) as a 30% by weight solution was added, followed by 14 g of wet-strength polymer Kymene® 557LX (Hercules Inc.) as a 12.5% by weight solution. Finally, 14 g of mordant poly(diallyldimethylammonium chloride) Nalco CP-261 (Nalco Corp.) was added as a 40 wt.% by weight solution. The mixture was diluted with water to give 25% by weight total solids.

The coating solution was coated on paper at 25°C using a hand-coating device with a Meyer rod so that the final dry thickness of the image-receiving layer was about 10 g/m². The paper was Carrara White Nokoosa Solutions Smooth, Grade 5128, Color 9220, (Georgia Pacific Co.) having a basis weight of 150 g/m². After the composition was coated, it was immediately dried in an oven at 60°C.

### Element 2 of the Invention

This element was prepared the same as Element 1 except that N-(2-aminoethyl)-3-aminopropylmethyldimethoxysilane (United Chemical Technologies, Inc.) was used instead of3-aminopropyltrimethoxysilane.

### Comparative Element C-1 (no amino-silane or wet-strength polymer)

This element was prepared the same as Element 1 except that 3-aminopropyltrimethoxysilane and Kymene® 557LX were not used.

### Comparative Element C-2 (no wet-strength polymer)

This element was prepared the same as Element 1 except that Kymene® 557LX was not used.

### Comparative Element C-3 (no amino-functionalized silane coupling agent)

This element is the same as Element 1 of the invention except that no amino-functionalized silane coupling agent was used.

### Printing

Images were printed on the above elements using a Hewlett-Packard Deskjet® 970 printer with ink cartridges 51645A (black) and C6578DN (color). The images comprised a series of rectangles of cyan, magenta, yellow, black, green, red and blue patches. Each rectangle was 0.8 cm in width and 20 cm in length.

### Density Test

Densities of the above patches were measured using an X-Rite® densitometer. There was no significant difference between the densities printed on Elements 1 and 2 of the Invention and Comparative Elements C-1, C-2 and C-3.

### Coating Strength Test

The strength of the image-receiving layer was tested by placing a piece of Scotch tape on the coating surface, and then pulling the tape off the coating gently with a consistent force. The coating strength was rated as follows:
Good = no material was taken off by the tape, or the tape could not be removed from the coating without tearing the paper
Fair = small amount of material was taken off by the tape
Poor = large amount of material was taken off by the tape

### Waterfastness Test

The waterfastness test was performed by placing one drop of water onto various color patches, waiting for 60 seconds, and then removing the water with a piece of tissue. The waterfastness was rated as follows:
Good = little or no color density change
Fair = slightly noticeable change in color density
Poor = large change in color density
The results are shown in the Table below.

**Table**

| Element | Coating Strength Rating | Waterfastness Rating |
|---|---|---|
| 1 | Good | Good |
| 2 | Good | Good |
| C-1 | Poor | Poor |
| C-2 | Fair | Fair |
| C-3 | Fair | Fair |

The above results show that the Elements of the invention had better coating strength and waterfastness as compared to the Comparative Elements.

## Claims

1. An ink jet recording element comprising a support having thereon an image-receiving layer comprising a polymeric network formed by a chemical reaction between a wet strength polymer, amino-functionalized inorganic particles, and a hydrophilic polymer other than a wet-strength polymer, wherein said wet-strength polymer contains at least one highly reactive group comprising an azetidinium or an epoxide, said amino-functionalized inorganic particles comprise silica gel, precipitated silica, or silicates and being obtainable by chemical bond formation between inorganic particles and an amino-functionalized silane coupling agent, and the hydrophilic polymer is poly(vinyl alcohol) present in the image-receiving layer in an amount of from 30 to 70% by weight, wherein the dry thickness of the image-receiving layer ranges from 5 to 30 µm.

2. The recording element of Claim 1 wherein said image-receiving layer contains other particles.

3. The recording element of Claim 1 wherein said amino-amino-functionalized silane coupling agent has the formula:
(R₁)ₓSi(OR₂)_{y}(R₃)_{z}
wherein:
each R₁ independently represents an alkyl or aryl group, and at least one R₁ is substituted with at least one amino group;
each R₂ independently represents an alkyl or aryl group;
each R₃ is an alkyl group;
x is from 1 to 3;
y is from 1 to 3;
z may be 0, 1 or 2; and
the sum of x, y and z is equal to 4.

4. The recording element of Claim 3 wherein said coupling agent is 3-aminopropyltrimethoxysilane or N-(2-aminoethyl)-3-aminopropylmethyldimethoxysilane.

5. An inkjet printing method comprising the steps of:
A) providing an ink jet printer that is responsive to digital data signals;
B) loading said printer with the ink jet recording element of claim 1;
C) loading said printer with an ink jet ink composition; and
D) printing on said ink jet recording element using said ink jet ink in response to said digital data signals.

## Patentansprüche

1. Tintenstrahlaufzeichnungselement mit einem Träger und darauf einer Bildempfangsschicht aus einem Polymernetzwerk, ausgebildet durch chemische Reaktion zwischen einem nassfesten Polymer, aminofunktionalisierten anorganischen Teilchen und einem hydrophilen Polymer, das kein nassfestes Polymer ist, worin das nassfeste Polymer mindestens eine sehr reaktionsfreudige Gruppe enthält, die Azetidinium oder ein Epoxid umfasst, wobei die aminofunktionalisierten anorganischen Teilchen Siliciumdioxid-Gel, ausgefälltes Siliciumdioxid oder Silicate umfassen und durch eine chemische Bindung zwischen anorganischen Teilchen und einem aminofunktionalisierten Silankupplungsmittel ausbildbar sind, und das hydrophile Polymer Poly(vinylalkohol) ist, das in der Bildempfangsschicht in einer Menge von 30 bis 70 Gew.-% vorhanden ist, worin die Trockendicke der Bildempfangsschicht zwischen 5 und 30 µm liegt.

2. Aufzeichnungselement nach Anspruch 1, worin die Bildempfangsschicht weitere Teilchen enthält.

3. Aufzeichnungselement nach Anspruch 1, worin das aminofunktionalisierte Silankupplungsmittel folgende Formel aufweist:
(R₁)ₓSi(OR₂)_{y}(R₃)_{z}
worin:
jeweils R₁ unabhängig für eine Alkyl- oder Arylgruppe steht und mindestens ein R₁ durch mindestens eine Aminogruppe substituiert ist;
jedes R₂ unabhängig für eine Alkyl- oder Arylgruppe steht;
jedes R₃ eine Alkylgruppe ist;
x für 1 bis 3 steht;
y für 1 bis 3 steht;
z für 0, 1 oder 2 stehen kann; und
die Summe von x, y und z gleich 4 ist.

4. Aufzeichnungselement nach Anspruch 3, worin das Kupplungsmittel 3-Aminopropyltrimethoxysilan oder N-(2-Aminoethyl)-3-Aminopropylmethyldimethoxysilan ist.

5. Tintenstrahldruckverfahren mit folgenden Schritten:
A) Bereitstellen eines Tintenstrahldruckers, der auf digitale Datensignale anspricht;
B) Beladen des Druckers mit dem Tintenstrahlaufzeichnungselement nach Anspruch 1;
C) Beladen des Druckers mit einer Tintenstrahltintenzusammensetzung und
D) Bedrucken des Tintenstrahlaufzeichnungselements mit der Tintenstrahltinte in Abhängigkeit von den digitalen Datensignalen.

## Revendications

1. Elément d'enregistrement par jet d'encre comprenant un support revêtu d'une couche réceptrice d'image comprenant un réseau polymère formé par une réaction chimique entre un polymère conférant une résistance à l'état humide, des particules inorganiques ayant une fonctionnalité amino et un polymère hydrophile autre que le polymère conférant une résistance à l'état humide, dans lequel ledit polymère conférant une résistance à l'état humide contient au moins un groupe hautement réactif comprenant un azétidinium ou un époxyde, lesdites particules inorganiques ayant une fonctionnalité amino comprennent du gel de silice, de la silice précipitée, ou des silicates, et pouvant être obtenu par la formation d'une liaison chimique entre les particules inorganiques et un agent de couplage au silane ayant une fonctionnalité amino, et le polymère hydrophile est un alcool polyvinylique présent dans la couche réceptrice d'image en une quantité variant de 30 % à 70 % en poids, dans lequel l'épaisseur à sec de la couche réceptrice d'image varie de 5 µm à 30 µm.

2. Elément d'enregistrement selon la revendication 1, dans lequel ladite couche réceptrice d'image contient d'autres particules.

3. Elément d'enregistrement selon la revendication 1, dans lequel ledit agent de couplage au silane ayant une fonctionnalité amino a la formule :
(R₁)ₓSi(OR₂)_{y}(R₃)_{z}
dans laquelle :
chaque R₁ représente séparément un goupe alkyle ou aryle, et au moins un R₁ est substitué avec un groupe amino au minimum ;
chaque R₂ représente séparément un groupe alkyle ou aryle ;
chaque R3 représente un groupe alkyle ;
x est compris entre 1 et 3 ;
y est compris entre 1 et 3 ;
z peut être égal à 0, 1 ou 2 ; et
la somme de x, y et z est égale à 4.

4. Elément d'enregistrement selon la revendication 3, dans lequel ledit agent de couplage est un 3-aminopropyltriméthoxysilane ou un N-(2-aminoéthyl)-3-aminopropylméthyl-diméthoxysilane.

5. Procédé d'impression par jet d'encre comprenant les étapes de :
A) fourniture d'une imprimante à jet d'encre sensible aux signaux de données numériques ;
B) chargement dans ladite imprimante de l'élément d'enregistrement par jet d'encre selon la revendication 1 ;
C) chargement dans ladite imprimante d'une composition d'encre pour jet d'encre ; et
D) impression sur ledit élément d'enregistrement par jet d'encre en utilisant ladite encre d'impression par jet d'encre en réponse auxdits signaux de données numériques.
